

May 3, 1938.

G. N. KIRSEBOM

2,116,245

## PREPARATION OF ALKALINE EARTH METALS

Filed Sept. 13, 1935



INVENTOR

Gustaf Newton <sup>INVENTOR</sup> Kiseboom

ATTORNEYS

## UNITED STATES PATENT OFFICE

2,116,245

## PREPARATION OF ALKALINE EARTH METALS

Gustaf Newton Kirsebom, Clifton, Bristol, England, assignor to Calloy Limited, London, England, an English joint-stock company

Application September 13, 1935, Serial No. 40,441  
In Great Britain September 21, 1934

6 Claims. (Cl. 75—67)

This invention is for improvements in or relating to the preparation of magnesium.

According to the present invention magnesium is prepared by heating an alloy thereof in a closed vessel to a temperature above the volatilization temperature of magnesium and condensing the metal vapour given off.

In its simplest form the invention consists in volatilizing the magnesium in a closed vessel from 10 a previously prepared alloy thereof with aluminium.

At the temperature required, e. g. 1200—1300° C. for carrying out the process of the invention, aluminium has an extremely destructive effect 15 upon any of the refractory crucibles or furnace linings employed. If, for example, the aluminium containing the alkaline earth material were simply heated externally in a crucible, the heavy costs entailed through the disintegration of the 20 crucible may make the process uncommercial.

It is therefore of great importance in carrying out the process of the invention to employ a method of heating, in which the heat is developed within the body of the metal itself and the crucible only becomes heated by conduction from the 25 hot metal.

One very convenient way in which the invention may be carried into effect is to heat the magnesium aluminium alloy in a high frequency 30 electric furnace lined with carbon or other suitable lining material.

For example; in carrying out the process, an aluminium-magnesium alloy may conveniently be prepared by the process described in United 35 States Patent dated 14th November 1933 No. 1,935,245 and such alloy may then be heated in a high frequency furnace without separating the alloy from the dross consisting of particles of alloy dispersed in aluminium oxide which is 40 formed in the reduction process.

It is not, however, necessary to prepare an aluminium alloy previously. On the contrary, metallic aluminium may be melted in a crucible with calcined magnesite or material containing 45 magnesium oxide in pieces of sufficient size to overcome the surface tension of the molten aluminium at a temperature above the volatilization point of the said alkaline earth metal. The aluminium will then reduce the magnesium oxide 50 and the magnesium formed alloys with the aluminium and simultaneously the magnesium will be volatilized and may be condensed in a suitable chamber. In this way the reaction may be continued until the bulk of the aluminium has been 55 converted to oxide.

The invention accordingly includes in combination the following steps:—

(a) Heating aluminium and magnesium oxide in a closed vessel above the volatilization temperature of magnesium, the magnesium oxide being in pieces of sufficient size to overcome the 5 surface tension of the molten aluminium.

(b) Condensing the alkaline earth metal vapour formed.

It is desirable, in order to be able to condense the magnesium without the formation of powder, to carry out the reduction process at a 10 temperature as near as possible to the volatilization temperature of magnesium.

The process of the invention has the great advantage that no hydrogen is required to prevent a reverse reaction and no special means are required for evacuating the apparatus before or during the reaction. The small amount of air which is initially contained in the closed chamber 15 in which the reaction is carried out reacts in the early stages of the process with the first magnesium formed, producing a small amount of oxide and nitride dust which does not interfere with the subsequent condensation of metal. 20

In carrying out the distillation the condensing 25 tube may be immersed in an oil bath and the condensed magnesium drops into this oil bath in large pieces, which after cleaning, may be easily melted together, e. g. under a flux or by other 30 means.

As the vapour pressure of aluminium at these 35 temperatures is practically nil, magnesium condensed in this way does not even contain traces of aluminium and is chemically pure in other respects.

It has sometimes been found useful to charge the crucible first with the calcined magnesite in pieces and to cover the charge with a disc, preferably of graphite, of somewhat smaller diameter than the crucible to allow space for molten metal to trickle down between the periphery of the disc and the sides of the crucible. Molten aluminium or aluminium-magnesium alloy is then poured in. The weight of the disc prevents the 45 calcined magnesite from floating up to the surface of the molten aluminium and in this way from the start of the reaction the magnesite is surrounded by aluminium ensuring thereby a quicker and more thorough reaction between the 50 pieces of magnesite and aluminium. After finishing distillation the still molten residual metal is removed from the dross by tilting the crucible with the disc in place.

Instead of using pieces of calcined magnesite,

briquettes of calcined magnesite and carbon may be employed.

The reaction between the calcined magnesite and aluminium will then first take place and the 5 briquettes will retain their form but will mainly consist of aluminium, aluminium carbide and aluminium oxide which may be worked up to aluminium. It is also possible instead of carbon to use other materials capable of forming bri- 10 quettes with magnesite.

In the practical working of the process for the manufacture of magnesium it has been found that magnesium does not sufficiently readily distil out of an alloy containing less than 8 per cent 15 magnesium. The distillation may therefore be conveniently carried out in such a way that 8 per cent aluminium-magnesium-alloy is used as starting material along with calcined magnesite, for example, in equal parts by weight. The mag- 20 nesium will distil off and this will go on until practically all the magnesium in the magnesite over and above what is required to maintain an 8 per cent alloy will distil over. When the rate of distillation slackens off, the remaining alloy 25 will contain 8 per cent magnesium approximately.

By working with a series of furnaces it is, therefore, possible on the large scale to use the 8 per cent aluminium-magnesium-alloy left over from one furnace by pouring it into the next 30 furnace along with the necessary fresh aluminium and calcined magnesite in lumps or pieces.

The system is then closed and distillation re-sumed until the rate of distillation again slackens off when the molten metal remaining in the 35 furnace and consisting of an aluminium-magnesium-alloy of approximately 8 per cent will be transferred to the next furnace in the series and so on. After the removal of the 8 per cent aluminium-magnesium-alloy from any furnace, the 40 dross will be removed and treated separately for the recovery of aluminium, the furnace then being ready for a new operation.

In carrying out the process on a commercial scale it is not practicable to conduct the con- 45 densed magnesium directly into an oil bath owing to the amount of oil volatilized and the danger of explosion, but provided air is kept out of the apparatus during the volatilization stage, it is possible to collect the condensed metal with- 50 out any serious losses in a chamber.

An arrangement of apparatus which has been found to work satisfactorily in practice is represented by the accompanying drawing in which Fig. 1 shows diagrammatically the arrangement 55 of the whole apparatus and Fig. 2 shows a modified form of oil seal.

Referring to Fig. 1 an ordinary injector furnace 1 is heated by an oil jet 2. In the furnace a graphite crucible 3 is placed which is long enough 60 to protrude above the top of the furnace.

The crucible is covered by a graphite lid 4. In the side of the crucible above the level of the top of the furnace, an opening 6 is made to which the condenser pipe 7 is attached by the graphite 65 and fireclay luting 5. The condenser pipe 7 leads into the top of a hood 8 standing in a shallow bath of oil 13. Inside the hood is a cylindrical receiver 9 in two parts held together by the tray 10 and the ring 11. The receiver 9 stands upon a ring 12 to raise it above the level of the oil 13 inside the hood. In the side of the hood a narrow tube 14 is fixed with its centre line in alignment with the centre of the condenser tube 7 and extending outward from the hood in a plane parallel with that of the condenser tube 7. The

end of this tube is a packing gland 17 through which a rod 16 passes and extends along to the bend in the condenser pipe 7. This rod is sealed with an oil seal at its lower end. In this pipe 14 there is also provided a narrow inlet pipe 16 which may be closed with a valve or rubber tube and clip.

In operation, magnesium oxide-containing material e. g. burnt magnesite is placed in the crucible 3 and molten aluminium filled into the crucible about half way. The system is then closed and the crucible heated to a temperature of 1200-1300° C.

The magnesium oxide is reduced and at the temperature of reduction it is volatilized off and condensed in the condenser tube 7. The condenser tube becomes heated by the heat of condensation to a temperature above the melting point of magnesium and the metal then melts and runs down dropping into the receiver 9. From time to time the rod 16 is moved to make sure that there has been no building up of condensed magnesium in the condenser tube 7 which may cause a blockage in the system. At the end of the run the furnace is shut down and as it cools, a reduced pressure is created in the hood 8. Enough air is allowed to enter through the inlet 16 to avoid oil being sucked up into the hood because if the oil comes into contact with the receiver 9 which is still quite hot, a rapid formation of oil vapour, which may lead to an explosion, results. It is found that the small amount of air that is required to be admitted in this way does not cause any appreciable amount of oxidation.

When the metal in the receiver has cooled sufficiently the hood is removed and the tray 10 and the ring 11 are knocked off the receiver 9 which is then broken apart.

Instead of the oil tray 10, a slightly modified form of oil lock is shown in Fig. 2. In this case the hood is closed with a disc 20 which is clamped to the bottom of the hood 8 by means of wedges 22 passing through eye-pieces 21 which latter are welded on to the sides of the hood 8 and pass through slots in the periphery of the disc 20. The hood 8 in this case is provided with a side tube 18 bent in the form of a U and dipping down into a small oil bath 19.

While the apparatus above described employs an oil fired furnace, it is, of course, preferable to employ a high frequency furnace for the reasons already set out.

The metal obtained as above described consists of large globules and prills separated by films of magnesium oxide and nitride. By simple melting under a flux such as carnallite a solid ingot of high purity may be produced.

I claim:—

1. A process for preparing metallic magnesium which comprises heating magnesium oxide at a temperature above the boiling point of magnesium with an aluminium-magnesium alloy containing about 8% of magnesium and condensing the metal vapour given off.

2. A process for preparing metallic magnesium which comprises heating together magnesium oxide with excess of aluminium by first charging pieces of magnesium oxide into a crucible and covering the said pieces with a loosely fitting graphite cover and pouring molten aluminium into the crucible and thereafter heating the molten aluminium and magnesium oxide above the volatilization temperature of magnesium.

3. A process as claimed in claim 2 wherein

there is employed instead of pieces of magnesium oxide brickettes thereof with carbon.

4. A process for preparing magnesium which comprises in combination the following steps:—

- 5 (a) heating magnesium oxide in a bath of molten aluminium in a closed vessel above the boiling point of magnesium, but below that of aluminium, the magnesium oxide being in pieces of sufficient size to overcome the surface tension of the molten aluminium and the amount of aluminium being sufficient to form an alloy with the reduced magnesium; (b) condensing the magnesium vapour formed.
- 10 5. A process as claimed in claim 4 wherein the reduction process is carried out at a tem-

perature just above the boiling point of magnesium.

6. A process for preparing metallic magnesium which comprises forming an alloy of magnesium with aluminium by heating together magnesium oxide with excess of aluminium at a temperature above the boiling point of magnesium whereby volatilization is effected simultaneously with the regeneration of the aluminium-magnesium alloy, and heating the aluminium-magnesium alloy in 10 a closed vessel to a temperature above the boiling point of magnesium and condensing the metal vapour given off.

GUSTAF NEWTON KIRSEBOM. 15